

## UNITED STATES PATENT OFFICE

2,407,881

PREPARATION OF GALVANIZED SHEETS TO  
RECEIVE RESINOUS COATINGSGeorge R. Hoover and Noble E. Hays, Middle-  
town, Ohio, assignors to The American Rolling  
Mill Company, Middletown, Ohio, a corporation  
of OhioNo Drawing. Application July 30, 1940,  
Serial No. 348,442

6 Claims. (Cl. 117—49)

1

Our invention relates to the preparation of ferrous sheets to receive resinous coatings, usually referred to as "baked enamels." Enamelled sheets and structures formed from sheets of this character are today widely used in industry—as one example, in the making of the cabinets of household refrigerators. For many uses galvanized sheets are desirable; and it has come to be the practice to give such sheets a pretreatment to promote their acceptance of the enamel and the bonding of the enamel to the sheets.

In the early days of the manufacture of baked enamel structures relatively little difficulty was encountered with blistering, though a number of complaints arose. The comparative unimportance of blistering was due to the substantially universal use of enamel substances of continuously thermoplastic character. More recently, however, there has been a shift to enamels which consist of resins of thermo-setting type, or contain large quantities of such resins; and blistering difficulties have become serious.

The principal objects of our invention are the solution of the blistering problem, and specifically the provision of a treatment for the sheets which is effective to prevent blistering.

It is an object of our invention to provide a treatment for the purpose which may be applied by the manufacturer of the sheets, and which produces a permanent effect so far as the sheets are concerned, so that blistering does not appear in spite of normal handling, shipping and storage conditions. It is our object to provide a treatment of such cheapness as not to add significantly to the cost of the sheets for enameling.

These and other objects of our invention which will be set forth hereinafter or will be apparent to one skilled in the art upon reading these specifications, we accomplish by that certain procedure and treatment and in that certain article of which we shall now describe exemplary embodiments.

The blistering problem is by no means confined to galvanized sheets which have been pretreated to promote acceptance and adhesion of enamels. Blistering upon ordinary galvanized sheets which have not been given any such treatment is also a problem and is equally amenable to the treatment which we hereinafter set forth. A galvanized sheet which has been "Bonderized" or given an adhesion and acceptance promoting treatment is, in our view, much more desirable for enameling use; and in the exemplary embodiment hereinafter taken up, we shall describe our process in connection with such a sheet.

2

Without desiring to be bound by theory we believe that blistering is caused by moisture and hydrogen coming from the sheet surface and failing to escape through the enamel. Formerly most of the enamels which were applied to metal parts and then heated to a drying temperature, contained, along with a suitable vehicle, thermoplastic resins which softened at the elevated drying or baking temperature but which increased the viscosity of the enamel vehicle sufficiently so that the enamel would not run off and produce too thin a coating. The elevated temperature had to be maintained until the vehicle polymerized and hardened. There was thus a considerable baking time during which the viscosity was not so high as to prevent the escape of any bubbles of entrained gas. In the newer types of enamel a thermo-setting resin is used which, with the vehicle, not only makes the enamel more viscous as applied, thereby yielding a heavier coating, but in itself undergoes a chemical change so that it hardens and becomes permanently infusible. This type of enamel has the advantage of setting much more quickly and attaining the maximum hardness after a shorter baking operation. It has the disadvantages of hampering the escape of bubbles of gas forming therein, of forming a film which tends to entrap the gases, and of hardening so rapidly as to prevent the escape of the gases. Resins of the thermo-setting variety which, along with suitable vehicles, constitute or are ingredients in the more modern types of baking enamels comprise generally resins of the urea-formaldehyde types, the phenol-aldehyde types, the glycerol-polybasic acid resins, the acetylene derivatives, and the poly-olefin resins. Enamels containing any of these resins present a blistering problem which is solved by the treatment of this invention.

40 In the formation of our improved sheets, the ferrous sheet metal is galvanized in any suitable way by being cleaned and treated with molten zinc or spelter, though we prefer to produce our galvanized sheets in accordance with the teachings of Patent No. 2,110,893.

45 The galvanized sheets are then passed through a solution containing phosphoric acid, zinc phosphate and an oxidizing agent such as sodium nitrate. This bath applies a coating of zinc phosphate to the sheet surface. The sheets enter the bath preferably through a set of rubber rolls kept wet with water, and they leave the bath through a set of rubber squeeze rolls which remove most of the phosphate solution from the sheet surface. Next they pass through a cold

water spray and then through a hot water spray in order to rinse off the remaining solution and any soluble salts which may be clinging to the sheet surface. Next, we prefer to pass the sheets through a set of rubber rolls into a chromic acid spray, being a solution of about three pounds of chromic acid per one hundred gallons of water at a temperature approximately 180° F. Finally they are passed through a set of squeeze rolls to remove the excess chromic acid solution and finally through a blast of hot air to dry the surfaces.

The treatment above is a treatment preferred by us for giving to the galvanized sheets an acceptance and adhesion promoting surface.

After extended research we have found that we can prevent the blistering of baked enamels as applied either to plain galvanized sheets or sheets which have been "Bonderized" as described above by giving to the sheets a heat treatment. Curiously enough, the effect of this heat treatment is permanent and the sheets after having once been freed of their tendency to produce blistering in baked enamels never regain that tendency, in spite of long periods of normal handling, shipping and storage.

The heat treatment to which we refer is a specialized heat treatment of which the most commercially available temperature range is from 450 to 500° F., within which temperatures the treatment can be completed in from 3 to 7 minutes or thereabouts. In investigating the effects of temperature we have found that heat treatments of temperatures as low as 250° F. will be effective if the time duration of the treatment is long enough, say 4 to 6 hours. Thus the lower limit of temperature is essentially a matter determined by manufacturing convenience and depending upon the lengths of time available for the heat treatment and the economics of relatively lengthy heat treatments. The upper limit of temperature is determined by the maximum temperature which will not adversely affect the adherence of the galvanized coating itself to the ferrous sheet. Different types of galvanized coatings will withstand different maximum temperatures. Certain galvanized coatings applied by the lead-zinc pot process have been known to begin to lose their adherence at below 500° F. Regular galvanized coatings can be heated to approximately 500 to 600° F. before adherence is damaged. Coatings made by the process of the patent referred to above can be heated much higher with entire safety, and can occasionally be heated as high as 900° F. for a short length of time before adherence is affected. Adherence tests for galvanized coatings are commonly used by manufacturers and in the light of these tests made at various temperatures the skilled worker in the art can readily determine the maximum permissible temperature for his particular product. Due to the shortness of the cycle (say 3 to 7 minutes) we recommend the temperature range of 450 to 550° F. for all galvanized products which will withstand these temperatures. If the skilled worker is working with a product which will not withstand these temperatures, he will be able in the light of the teachings above to select a time of treatment consonant with a temperature low enough not to affect the adhesion of his galvanized coating.

Our treatment therefore is effective in producing a galvanized sheet which as manufactured has no tendency to produce blistering with the

modern baked enamels and which, unobviously, is permanent in this respect.

The heat treatment may be carried out in a variety of ways because the sheets may be treated either singly or in packs. Where the time cycle is short enough to permit it, the sheets may be passed singly or in groups through an open heat treating furnace equipped with a conveyor (or strip may be pulled through the furnace) or the sheets (or coils) may be stacked on a platform, covered with a box or not as desired and heated in any suitable heat treatment apparatus capable of maintaining the desired temperature for the desired length of time.

15 Modifications may be made in our invention without departing from the spirit of it. Having thus described our invention, what we claim as new and desire to secure by Letters Patent is:

1. A process for the treatment of galvanized 20 ferrous articles including steps to free them from a blistering tendency when coated with thermosetting enamels, which comprises heat treating the galvanized sheets at a temperature and for a time sufficient to destroy the blistering tendency, but below a temperature and time cycle at which 25 adherence of a galvanized coating will be adversely affected, and hence without altering the extent of alloy formation, said temperature being applied by passing the articles through a continuous heat treating furnace and subjecting them therein to a temperature of from 450 to 550° F. for from 3 to 15 minutes, the time duration of the 30 heat treatment varying substantially inversely to the temperature thereof, and thereafter coating the articles with a thermosetting enamel.

2. A process of preparing galvanized sheets for the reception of baked enamels containing thermosetting resins and of destroying the tendency of said sheets to produce blistering, which 40 comprises galvanizing the sheets, giving the sheets an acceptance and adhesion-promoting treatment involving the formation of an insoluble zinc compound on their surfaces, and thereafter heat treating the sheets but below a temperature and 45 time cycle at which adherence of a galvanized coating will be adversely affected, and hence without altering the extent of alloy formation, by passing them through a continuous annealing furnace and subjecting them to a temperature of 450 to 550° F. for from 3 to 15 minutes, the time duration 50 of the heat treatment varying substantially inversely to the temperature thereof.

3. The process as claimed in claim 2 in which 55 said acceptance and adhesion-promoting treatment comprises treating the galvanized sheets with a solution of phosphoric acid, zinc phosphate and an oxidizing agent, thereafter washing said sheets, treating said sheets with a chromic acid solution, and drying said sheets.

4. A process for the treatment of galvanized 60 ferrous articles including a treatment to free them from a blistering tendency when coated with thermosetting enamels, which comprises heat treating the galvanized sheets at a temperature 65 and for a time sufficient to destroy the blistering tendency but below a temperature and time cycle sufficient to impair adhesion of a galvanized coating and hence without substantially altering the extent of alloy formation, the temperature of 70 said heat treatment lying substantially within the range of 250 to 600° F. and the time lying substantially between 3 minutes and 6 hours, the time duration of the heat treatment varying substantially 75 inversely to the temperature thereof,

and thereafter coating said articles with a thermosetting enamel.

5. A process of preparing galvanized iron and steel sheets for the reception of baked enamels containing thermosetting resins and of destroying the tendency of said sheets to produce blistering, which comprises galvanizing the sheets, giving the sheets an acceptance and adhesion-promoting treatment involving the formation of an insoluble zinc compound on their surfaces and thereafter heat treating the sheets in a temperature and time cycle below that at which adherence of the galvanized coating is impaired and hence without substantially altering the extent of said alloy formation, said heat treatment being at temperatures substantially within the range of 250 to 600° F. for from substantially 3 minutes to substantially 6 hours, the time of heat treatment varying inversely to the temperature thereof.

20

6. A process of preparing galvanized iron and steel sheets for the reception of baked enamels containing thermosetting resins, and of destroying the tendency of said sheets to produce blistering, which comprises galvanizing the sheets, giving the sheets an acceptance and adhesion-promoting treatment involving the formation of an insoluble zinc compound on their surfaces and thereafter heat treating the sheets in a temperature and time cycle below that at which adherence of the galvanized coating is impaired and hence without substantially altering the extent of alloy formation, said heat treatment being at a temperature of substantially 250° F. for substantially 6 hours, the said sheets being stacked on a platform and covered with an annealing box.

GEORGE R. HOOVER.  
NOBLE E. HAYS.